

## UNITED STATES PATENT OFFICE

1,988,012

## METAL DEPOSITS IN OXIDE COATINGS

Ralph Bryant Mason, New Kensington, Pa., assignor to Aluminum Company of America, Pittsburgh, Pa., a corporation of Pennsylvania

No Drawing. Application October 27, 1932  
Serial No. 639,850

9 Claims. (Cl. 148—6)

This invention relates to the production of decorative coatings on aluminum and aluminum alloy surfaces and it is particularly concerned with a method of producing on such surfaces decorative 5 coatings in which the color effects are obtained by the deposition of metal.

Numerous recently-developed methods of producing coatings which consist substantially of aluminum oxide on the surfaces of aluminum and 10 aluminum base alloys have extended the application of these metals to various uses and to the production of various articles for which they were heretofore considered unsatisfactory. These so-called oxide coatings, being dense and adherent, 15 protect the surfaces of the metal from corrosion and, being more or less porous and adsorbent, lend themselves to the production of decorative effects on metal surfaces by the coloring of the oxide coating.

20 It is an object of this invention to provide a new and improved method for the treatment of such oxide-coated aluminum and aluminum alloy surfaces to produce colored coatings having properties heretofore unknown in such coatings whereby 25 the utility of the coatings is further increased and they are made applicable to numerous new uses.

It is more particularly an object of this invention to provide a method for treating oxide-coated aluminum and aluminum base alloy surfaces to 30 produce metallic deposits therein.

My invention is predicated upon the discovery that if an aluminum or an aluminum alloy surface provided with an oxide coating be treated with 35 solutions of one or more of a certain class of metallic salts and with a reducing agent the metallic salt may be reduced in situ and the deposit of free metal obtained in and on the oxide coating. The metallic deposit thus produced imparts to the oxide coating a characteristic color 40 and it modifies the properties of the coating by increasing its corrosion resistance and by imparting to it the property of conducting electricity, although its resistance may be high. This combination of properties has heretofore been unknown in such coatings, as the oxide coatings themselves are generally considered to be excellent 45 electrical insulators.

In carrying out my invention the oxide coating 50 may be produced upon the aluminum or aluminum alloy surface in any suitable manner whereby there is obtained a relatively hard, porous, adherent and adsorbent coating. For this purpose I have found that anodic oxidation of the aluminum or aluminum alloy surface in an electrolytic

cell, using as an electrolyte a solution of an acid such as sulfuric acid, chromic acid or oxalic acid, is particularly suitable, but satisfactory results may also be obtained by numerous other methods, such for example as by simple immersion of the aluminum article in a solution of sodium carbonate and potassium dichromate or similar oxidizing solution without the application of electrical energy. Anodic oxidation is to be preferred, however, as harder, more adherent coatings 10 possessed of better adsorbent properties are produced. Particularly good results may be obtained by making aluminum or aluminum base alloy articles to be coated the anode in an electrolytic cell, using as the electrolyte a solution of sulfuric acid. The conditions of temperature, time and current density used for the oxidation vary with the concentration of the electrolyte used, and when using sulfuric acid electrolytes, concentrations of about 1 to 70 per cent acid may be used. 15 A satisfactory adsorbent and adherent oxide coating may, for example, be obtained by anodic oxidation of the aluminum article in a solution of 7 per cent sulfuric acid by the application of a current of 0.01 to 0.4 amperes per square inch of 20 anode surface for about 30 minutes at room temperature.

After a suitable oxide coating has been formed on the aluminum or aluminum alloy surface the coated metal is treated according to my invention 30 to produce a metallic deposit therein. The metallic deposit is obtained by treating the oxide-coated metal successively with a solution of a reducible metallic salt and a solution or other suitable form of reducing agent. The reducible 35 metallic salts must be such salts as are soluble and more or less reducible in solution, and they must be capable of complete reduction to the metal. The salts of the metals of the subgroup of group 1 of the Mendelejeff periodic system, copper, silver and gold, sometimes designated as the copper group metals, have been found to possess these properties in a high degree and are particularly adaptable to use in the coloring of oxide coatings 40 according to my invention, but other suitable metal salts may be used. The reducing agent used may be either in the form of a reducing solution or a reducing gas, or in any other adsorbable form, although it is usually preferable to use the 45 reducing agent in solution. The oxide-coated aluminum is treated with the solution of the reducible metallic salt and with the reducing agent so that these reactants are adsorbed in and on the oxide coating whereby the reducing reaction is 50 55

produced within and on the oxide coating. The reducing action thus obtained deposits finely divided metal within and on the oxide coating.

The metallic deposits thus produced have characteristic colors which are useful for decorative purposes and which vary with the salts from which they are deposited and the method of their deposition. The metal deposits are usually in the state of division approaching colloidal size, and with variation in the size of the particles deposited variance in the shade of the characteristically-colored deposits is produced. For example, deposits of silver may be produced having the characteristic color of colloidal silver varying in shade from brown to brownish black. Various shades of reddish purple colloidal gold deposits may also be obtained in this way, as well as yellow colored deposits of colloidal copper. The particular shades obtained vary with the salt of the metal first deposited, with the concentration of the solutions used, and with the particular reducing agent applied and its method of application.

In producing silver deposits the oxide coating may be first impregnated with a solution of substantially any soluble silver salt, but silver nitrate solutions have been found to be preferable. Particularly satisfactory for this purpose are alkaline solutions of silver nitrate in ammonium hydroxide, the salt in this form being readily reducible to the metal. The concentration of the salt solution may vary between wide limits, depending upon the results desired, but it is generally preferable to use solutions containing about 1 to 20 per cent of the salt. The reduction of the silver salt is accomplished preferably by immersion of the impregnated oxide coating in a solution of a reducing agent. Solutions of reducing sugars, pyrogallic acid, hydroquinone, hydrazine sulfate, formaldehyde, tannic acid, or mixtures of these reducing agents may, for example, be used. The reduction may also be made by treatment of the solution-impregnated oxide coating with a reducing gas, such as by treatment with formaldehyde gas. The color of the metallic deposit obtained may be varied by reversing the order in which the solutions of reducible metallic salt and the reducing agent are applied to the oxide coating, and in using certain types of metallic salts it is preferable that the order of application of these solutions be reversed from that usually applied. For example, when a simple solution of silver nitrate in water is used it is usually preferable to treat the oxide-coated aluminum surface first with the solution of the reducing agent and subsequently with the solution of the reducible metallic salt, as better results are obtained thereby.

Copper deposits may be produced from solutions of salts similar to those used for depositing silver. Tannic acid and hydrazine sulfate solutions have been found particularly useful for use as reducing agents in conjunction with a solution of ammoniacal copper sulfate. Gold chloride solutions, preferably alkalized with potassium carbonate, may also be used in conjunction with tannic acid, formaldehyde or other reducing agents to produce deposits of gold.

In the following examples, there are set out more specifically the results which may be obtained by my process, and the variations in color and shade resulting from varied conditions of operation.

### Example 1

An aluminum sheet was first provided on its surface with an adherent and adsorbent oxide coating by subjecting it, as the anode, to the action of a 7 per cent sulfuric acid solution in an electrolytic cell, using a current density of 0.08 amperes per square inch of anode surface. An ammoniacal solution of copper sulfate was prepared by adding concentrated ammonium hydroxide to a solution of copper sulfate until the precipitate formed was just re-dissolved. This solution was diluted to a concentration of about 10 per cent. As a reducing solution, 0.5 grams of hydrazine sulfate was dissolved in 200 cc of water and about 0.5 per cent of caustic soda was added. The oxide-coated sample was immersed in this solution of ammoniacal copper sulfate and then, after rinsing, in the water solution of hydrazine sulfate. A yellow deposit of finely divided copper was thus obtained.

### Example 2

A sample of aluminum sheet was first provided with an oxide coating as described above in Example 1. A solution of 1 per cent silver nitrate was prepared, to which a small amount of potassium hydroxide was added. Sufficient ammonia was then added to just re-dissolve the precipitate formed. A reducing solution of hydrazine sulfate was prepared as described in Example 1. The oxide-coated aluminum sample was first immersed in the ammoniacal silver nitrate solution, rinsed, and then immersed in a hydrazine sulfate solution. A brown deposit of colloidal silver was obtained.

### Example 3

An oxide-coated aluminum article was first immersed in a solution containing 2.5 per cent pyrogallic acid and 2.5 per cent sodium thiosulfate or hypo. The article was then rinsed and immersed in a 10 per cent solution of silver nitrate. A very dark brown to black silver deposit was obtained.

### Example 4

A reddish purple color was obtained by depositing gold, in a colloidal or semi-colloidal state of division, in an oxide coating. In producing this color the aluminum article, provided on its surface with an oxide coating, was first impregnated with a 10 per cent solution of tannic acid. The impregnated coating, after rinsing, was then immersed in a solution of gold chloride containing 0.6 per cent of the salt, to which had been added 3 per cent of potassium carbonate.

The colored oxide coatings thus obtained are substantially permanent and are very suitable for decorating aluminum surfaces, particularly such surfaces as are to be used in exposed positions. In some cases, however, particularly where the lighter colored silver deposits are obtained, there is a tendency for such coatings to change color with exposure to sunlight. This effect may be due to the fact that in such cases a certain amount of un-reduced or partially reduced metallic salt remaining in the coating is reduced by the action of the sunlight. The term "metal deposits" as it has been used throughout this specification must, therefore, be understood to include not only deposits of completely reduced metal but also such mixtures of metal and un-reduced or partially reduced metal salts as may be obtained by practicing my invention according to the above description.

Having now particularly described and pointed out my invention, what I claim is:

1. A method of coloring aluminum or aluminum alloy surfaces comprising producing on such surfaces an adherent and adsorbent oxide coating and treating said coating successively with a solution of a reducible metallic salt and with a reducing agent.
2. A method of coloring adsorbent oxide-coated aluminum or aluminum alloy surfaces which comprises impregnating said oxide coating with a reducible metallic salt and treating said impregnated oxide coating with a reducing agent.
3. A method of coloring adsorbent oxide-coated aluminum and aluminum alloy surfaces which comprises depositing finely divided metal therein by treating said coating successively with a solution of a reducible metal salt and with a reducing agent.
4. A method of coloring adsorbent oxide-coated aluminum or aluminum alloy surfaces which comprises impregnating said surfaces with a solution of a soluble salt of a metal of the group consisting of copper, silver and gold and with a reducing agent.
5. A method of coloring adsorbent oxide-coated aluminum or aluminum alloy surfaces which comprises impregnating the oxide coating with a solution of an ammoniacal silver nitrate and treating said impregnated oxide coating with a reducing agent.
6. A method of coloring adsorbent oxide-coated aluminum or aluminum alloy surfaces which comprises impregnating said oxide coating with a solution of a reducing agent and subsequently treating said impregnated oxide coating with a solution of a soluble silver salt.
7. A method of coloring adsorbent oxide-coated aluminum or aluminum alloy surfaces which comprises treating said surfaces successively with a solution of a soluble copper salt and with a reducing agent.
8. A method of coloring adsorbent oxide-coated aluminum or aluminum alloy surfaces which comprises treating said coating successively with a solution of a soluble gold salt and with a reducing agent.
9. A method of coloring aluminum or aluminum alloy surfaces comprising producing on such surfaces an adherent and adsorbent oxide coating, and treating said coating with solutions of a reducible salt and a reducing agent capable of reducing said salt, by first absorbing material from one of said solutions in the coating and then treating with the other solution.

RALPH BRYANT MASON.